

May 6, 1952

W. W. ODELL ET AL

2,595,365

CARBONIZATION OF CARBONIZABLE SOLIDS

Filed June 14, 1947



William W. Odell Inventors  
George L. Matheson  
By L. F. Tracy Attorney

## UNITED STATES PATENT OFFICE

2,595,365

## CARBONIZATION OF CARBONIZABLE SOLIDS

William W. Odell, Washington, D. C., and George L. Matheson, Union, N. J., assignors to Standard Oil Development Company, a corporation of Delaware

Application June 14, 1947, Serial No. 754,623

5 Claims. (Cl. 202—6)

1

This invention relates to the carbonization of solid fuels. It has to do with the carbonization of solid carbonizable materials by subjecting them to an elevated temperature while in a fine state of subdivision. More specifically it relates to the carbonization of finely divided solid fuels and the production therefrom of finely divided carbonized solids by passing the said finely divided fuel as a stream while confined in a carbonizer downwardly through a hot zone at a controlled rate while promoting combustion in said zone in contact with said solids and while passing a gasiform stream upwardly through said downwardly flowing fuel solids at such a velocity that the particles of solid fuel in process are maintained as a fluidized state in said carbonizer. The invention relates to both process and apparatus whereby the finely divided solid fuel prepared for carbonization is in part deashed prior to its passage through the hot zone.

In ordinary practice in carbonizing solid fuels, the employment of very finely divided fuels is avoided usually because a stationary bed of such solids forms a heat insulating mass which results in prolonged duration of the time of carbonizing. So far as we are aware, it has not been economical to treat finely divided solids for the purpose of making a finely divided carbonized solid residue. Our experiments show that a solid fuel can be economically carbonized in a fine state of subdivision, provided means are supplied for fluidizing it and passing it in the fluidized state in countercurrent direction and in contact with upwardly flowing hot gases. It has also been found desirable to control the temperature in the hot zone of the fluidized fuel in the process and to control its rate of travel through the hot zone, as well as to control the nature of the hot gases with which it is contacted during processing.

One of the objects of this invention is to carbonize finely divided solid, carbonizable fuels rapidly. Another object is to control the duration of the carbonizing time, the temperature of carbonization, and the nature of the fluidizing gas streams employed so that the product of carbonization is highly reactive and may be called an activated carbon. Another object is to recover gaseous and vaporous products from the carbonization of finely divided solid fuel. Still another object is the reduction of the ash content of the fuel prior to its carbonization. Another object is to provide apparatus in which the aforementioned objects can be accomplished economically. Still other objects will become

apparent from the disclosures hereinafter made.

In the carbonization of coal, it is necessary to take into consideration the condition of the coal other than its state of fineness. The coal rank and amount of exposure of the coal to the atmosphere have much to do with coking properties of coal. Considerations are given to these factors in the operation of the process of this invention. It is well known that lignite, sub-bituminous coal, and certain bituminous coals do not have strong coking properties and, therefore, they can be readily carbonized in a fine state of division without appreciable agglomeration or building up of large size pieces by cementation. However when coals having strong coking properties are ground to fine sizes and are directly carbonized by exposure to heat, the coal passes through a plastic state at a temperature of approximately 800 to 860° F., and it is necessary in order to obtain an end product, which is also in a fine state of sub-division, to prevent the agglomeration of particles or to reduce agglomerating action to a minimum. We find that this can best be done when the particles of coal in process are maintained in the fluidized condition during the heating period and particularly during that period in which they pass through the plastic range of temperature. By maintaining particles during carbonization in vibrant or ebullient motion, it is found that carbonization can be so conducted that the solid residue is in a fine state of subdivision. Our tests also reveal that it is desirable to maintain the particles of solid fuel in a violent state of ebullient motion in the presence of similar solids which have already been carbonized, while they pass through the plastic range of temperature. When carbonization has once taken place at the chosen temperature, say for example 700° C. (1292° F.) activation is promoted by passing steam through the fluidized carbonized mass, thus activating and cooling simultaneously. Means for accomplishing these ends are provided in this invention as will become evident by reference to the figure.

The single figure in the accompanying drawing is a diagrammatic elevation of one form of apparatus which can be used in the carbonization of solids according to this invention and it shows rather schematically a flow diagram of the fluids and solids employed.

In the figure the carbonizer 1 confines a bed of fluidized solids having a top level L and it has packed zones 2 and 3, which zones contain non-fluidized solids of much larger size than the par-

ticles of fuel to be treated and which solids form a porous bed or mat, the interstices of which are channels for the passage of the finely divided particles of fuel downwardly therethrough and for the upward passage of gases therethrough. The carbonizer has a porous support 4 for the bed of fluidized solids, an outlet 5 with control valve 6 for the discharge of the fluidizing stream, and a dust separator 7.

Located adjacent to the top of the carbonizer 1 and connected thereto is a de-ashing unit 10. This unit is preferably identical in construction and mode of operation with that described in our co-pending application Serial No. 726,530, filed February 5, 1947, now abandoned and entitled "Process and Apparatus for Separating Mixed Materials." A similar system is described and claimed for the production of activated carbon in our copending application Serial No. 754,624, filed June 14, 1947, and entitled "Processing Carbonaceous Solids." For the purpose of this description it is sufficient to note that near its lower end, the de-ashing unit is provided with a porous grid or grate 11 below which is an inlet line controlled by valve 24 for introducing a fluidized gas which may be air or combustion gas or any other gas which is preferably not reactive with the solid material treated in this zone. The de-ashing unit is operated so as to maintain therein a level of fluidized solid L1, which is sufficiently high to cause the solid to overflow into the drawoff line 28 controlled by valve 29. This drawoff line terminates in the carbonizer 1 below the level L of the fluidized solid therein.

At the upper end, the de-ashing unit is provided with a line 12 for leading off the fluidizing gas. The flow of this line is controlled by a valve 13. Connected with line 12 is branch line 15 which may be used to conduct the fluidizing gas, where it is air, oxygen or other combustion supporting gas, to bustle pipe 16 which is connected to the carbonizer 1 between zones 2 and 3. The flow of gas in branch line 15 is controlled by valve 14. At an intermediate point the de-ashing unit is provided with inlet line 34 controlled by valve 33 through which the finely divided solid fuel to be treated is introduced into the unit. At its lower end, above the grid 11 the unit has a drawoff line 26 controlled by valve 27 for withdrawing ash from the unit.

When reference is made to ash in connection with this de-ashing unit, there is contemplated those non-fuel materials with which the fuel matter is contaminated such as quartz, sand, shale, gypsum, pyrites and other mineral matter. This ash has a density greater than the fuel material whereby when the de-ashing unit is operated in accordance with the teachings of our aforesaid application, a fairly complete separation of the fuel constituents from the ash can be realized with the fuel constituents leaving the unit near the top thereof and the ash leaving the unit from its bottom portion.

Combustion supporting gas, which may be air, is supplied through conduit 18 and valve 19 to the combustion zone 17 of the carbonizer, whereas said combustion supporting gas is supplied when desired also through conduit 20, valve 21 and inlet 23 to the base of the carbonizer. Steam is introduced through valve 22 and intake 23. Means for withdrawing the treated solids, namely the carbonized finely divided solids, from the carbonizer, are indicated by offtake 31 and valve 32. Auxiliary means of supplying a gasiform stream to the carbonizer at an upper zone thereof is

shown by conduit 9 and valve 8; the stream may be a combustion supporting fluid, steam, gas such as recycle gas, mixtures thereof, or other gaseous material, according to effect desired.

Referring to the figure, the operation, in general, is as follows: Finely divided solid fuel to be treated is charged into a middle portion of the re-ashing unit 10 through valve 33 and conduit 34 at a rate adapted to maintain the bed level L1 in said unit. Air or other fluidizing gas is introduced through 24 and passes through porous member 11, fluidizing the finely divided fuel in 10, the gas stream passing out through 12, at least a portion of it being conducted through valve 14 and conduit 15 to carbonizer 1, whereas the remainder, if any, is discharged through valve 13. The fuel thus fluidized in 10 separates from a portion of its ash content, the ash passing out through offtake 26 and valve 27, whereas the de-ashed fuel is discharged substantially continuously through offtake 28 and valve 29 to the carbonizer 1.

Steam is introduced into carbonizer 1 through valve 22 and conduit 23, and combustion is promoted in the hot zone 17, after some of the fuel in this zone is ignited, by virtue of combustion supporting gas supplied through bustle pipe 16 to said hot zone. Valve 32 is opened sufficiently to allow treated solids to pass out of carbonizer 1 through offtake 31 at a predetermined rate. The products of the combustion promoted in hot zone 17, along with the gases resulting from passing steam up through the fluidized solids in the portion of the carbonizer below the hot zone, pass upwardly through the packed zone 2 and the upper fluidized zone A at such a rate that the particles of said fuel are maintained in vibrant or ebullient motion throughout the bed. Some of the heat generated by the combustion in zone 17 is imparted to the downwardly moving fluidized solid fuel of which the bed is comprised.

After operations are underway, it will be found that the steam entering through intake 23 absorbs heat from the solid fuel in the lower portion of the fluidized solids in carbonizer 1 and to some extent in cooling the carbonized product it reacts therewith forming hydrogen and carbon oxides, which gases further react in the combustion zone 17. Thus the finely divided solid fuel is heated to a temperature above the plastic range in the upper portion of the bed in carbonizer 1 and it then passes through a hotter zone in contact with the non-fluidized solids 2 and finally through the hottest zone 17 of the bed wherein it reaches the chosen maximum temperature and then passes through packed zone 3 and zone C which are the steaming and activating zones, discharging as described through 31 and 32.

Thermocouples indicated by 38 and 39 are employed to aid in regulation of the operation. Sufficient combustion is promoted in combustion zone 17 so that the gas stream passing up through the packed zone 2 and through the upper fluidized portion of the bed in zone A, has a temperature sufficiently high to heat the fluidized particles in zone A to a temperature above the plastic limit so that clogging will not occur as these particles are drawn downwardly into the packed zone 2. Since it is usually desirable to maintain a given maximum temperature in the combustion zone 17, it is sometimes desirable to recirculate products of combustion or other diluent gasiform stream with the air supplied to

## 5

carbonizer 1 through 16 in order to prevent excessively high temperature in zone 17 and in order to furnish a sufficient volume of hot gas to accomplish the desired fluidizing and heating effect in zone A.

In making active carbon, it is usually desirable that the particles of the carbonizable material treated be heated suddenly to a temperature of the order of 900° to about 1200° F., and that the product resulting from this heating be subsequently heated to a higher temperature and subsequently steamed. All of these are accomplished in the operation of the carbonizer 1 of the figure as described. The hot particles passing from zone 17 downwardly through the packed zone 3, contact steam rising through zones C and 3 and form a given amount of water gas, which gas is burned in zone 17. Thus a portion of the heat required for conducting the process is furnished by the steaming which is essential in making activated carbon. The operation, with modifications to suit special conditions, is applicable to the production of bone black from crushed bones, to the production of a carbonized fuel suitable for use in making briquettes or in mixtures with coking coal for coke-oven use and for otherwise treating materials which require heating to elevated temperatures and cooling.

An example of the production of activated carbon with yields obtained in a particular case are given as follows: Raw lignite is used as the raw material and it is crushed to a size of 20 mesh with some smaller sizes. It is then passed through an ash separator as shown at 10 in the figure, and the ash content is reduced. During this de-ashing the lignite is dried by passing hot gases up through the de-ashing unit. The warm partly de-ashed lignite in a fine state of division is substantially continuously discharged from the unit 10 through offtake 28 and valve 29 to the carbonizer 1 into the fluidized bed of similar but hot partially carbonized lignite, which bed is at a temperature of 1200° F. This temperature is maintained in the upper zone A. Meanwhile the volatile matter and tarry vapors are discharged from above the bed through separator 7, offtake 5 and valve 6. The tarry vapors are condensed and separated by known means.

The solid particles of lignite are carbonized in the fluidized state and are substantially continuously passed downwardly from the top zone of the bed to substantially the bottom zone of the bed, namely from zone A to zone C. Combustion is promoted in a middle zone 17 of the carbonizer, whereby the temperature is maintained therein at 1470° to 1650° F. The combustion is promoted in zone 17 by passing the air used for fluidizing the solids in de-ashing unit 10 back through valve 14, conduit 15 and bustle pipe 16 into the carbonizer 1. Throughout this operation steam is introduced from beneath grid 4 through valve 22 and inlet 23. The solids resulting from carbonization, which under these conditions is an active carbon, is withdrawn substantially continuously through offtake 31 and valve 32.

The temperature in the upper zone A of the fluidized bed in the carbonizer 1 preferably should be in the range 1000° to 1250° F. for the production of carbon for use in removing sulfur from gases for example. The amount of combustion promoted in zone 17 is that which will provide the desired temperature in the upper zone A and at the same time raise the temperature of the particles passing through 17 to a tem-

## 6

perature of the order of 1450° to 1850° F. usually. The steam passing through 22 and 23 partly cools the carbon in zones 3 and C, and simultaneously generates gas by the water gas reaction. The gas stream introduced into the carbonizer through pipe 16 is the major fluidizing-stream component, whereas in the lower portion of the bed, namely in zones 3 and C, the steam is the major fluidizing reactant. For the purpose of fine adjustment of temperature, some air can at will be introduced along with the steam by opening valve 21 to a desired extent. Likewise other fluidizing medium than the circulating gas can be introduced through 16 by opening valve 19.

The raw lignite treated as above has a composition substantially as follows:

|              | Per cent by weight |
|--------------|--------------------|
| Moisture     | 32.4               |
| Volatile     | 26.4               |
| Fixed carbon | 32.8               |
| Ash          | 8.4                |
| Total        | 100.0              |

B. t. u. per pound 7,310

The composition after drying and de-ashing is:

|              | Per cent by weight |
|--------------|--------------------|
| Moisture     | 0.3                |
| Volatile     | 41.7               |
| Fixed carbon | 51.7               |
| Ash          | 6.3                |
| Total        | 100.0              |

The ash removed per ton of raw coal used was 88 pounds or 52.3 per cent of the ash originally present. The partly carbonized lignite as it leaves zone A and passes into the packed portion, zone 2, is largely carbon with 5 to 7 per cent of volatile matter, the remainder being ash. The yield at this point is a little more than 35 per cent of the total raw lignite treated. The calorific value is about 12,600 B. t. u. per pound. The tar evolved amounts to about 5.6 gallons per ton of raw coal treated. The specific gravity of the tar is about 0.98. The approximate gas yield per ton of raw lignite treated at this particular temperature, and separately determined, without dilution with other gases, is about 4470 cubic feet. The yield of activated carbon after passing through zones B and C is approximately 29 per cent of the original lignite used.

The properties of carbon made in this manner vary according to the nature of the raw material initially charged to the rate of heating of the upper zone A, to the final temperature attained in the hot zone 17, and to the amount of steaming, as well as the temperature of the steam introduced through valve 22 and intake 23. These variables can be adjusted to suit any particular case.

It is essential that the particles of lignite in process be sufficiently fluidized so that they will mix and will flow downwardly through the packed zones as described. The factors relating to velocity of flow for given size particles is now well known in the art but for the purpose of clearness it may be stated that with particles having sizes as given in the foregoing example, the velocity of the fluidizing stream as it leaves the bed of fluidized solids in carbonizer 1 should be approximately 0.4 to 1.0 feet per second; finer size solids do not require as high a velocity of the fluidizing stream as large size particles.

It is important that the size of the packing in zones 2 and 3 be sufficiently large so that the interstices are large enough for the particles of solids being treated to be fluidized therein and flow downwardly therethrough.

It will be understood that the temperature in zone 17 may be controlled to suit conditions and may be as high as 2200° F., although it is commonly within a range of 1400 to 1800° F. It is also understood that the steam may be superheated as the occasion requires.

It is further understood that the gases removed through offtake 5 and valve 6 from the carbonizer may be used, after removing condensable matter therefrom, as fuel, and supplied to zone 17 by means not shown, or through conduit 18 and valve 19 when so desired. Similarly the latter gas or gas passing out through valve 13 may also be introduced with the steam beneath grid 4 when desired.

When using strongly coking coals as the raw material to be carbonized, it has been found that the introduction of an auxiliary heating fluid in zone A of the bed above the packed zone 2 is sometimes beneficial. This not only has the effect of decreasing the bed density in zone A but it permits the introduction of some oxygen, which may be in the form of air, with or without steam or recirculated gas; its use facilitates the heating of the particles in zone A and minimizes any tendency for particle agglomeration, although it does tend to reduce the amount of readily recoverable tar produced. When it is desirable to increase capacity to the maximum, air can be thus introduced through valve 8 and conduit 9, or air with recirculated hot gas may be used with steam as desired.

Other modifications of operating procedure may be conceived within the scope of this invention and likewise novel effects may be produced by a different arrangement of packing zones than those shown in the figure. A greater number of packed zones than two may be employed and the packing material used may be spheres, Berl saddles, or other shaped material which will resist exposure to heat and which will furnish satisfactory interstitial space for the flow of particles in process therethrough. The duration of the time of exposure of the carbonized particles in zones 3 and C to the action of steam is controllable by controlling the size of the chamber confining these zones, particularly the depth.

Referring to the figure, operating adjustments are made, after the rates of flow of feed of fresh solids, discharge of treated solids and supply of fluidizing medium are once set, as follows: To increase the completeness of carbonization of the solids flowing into zone B from zone 2 either decrease the rate of feed of solids by adjusting valve 29 and similarly adjusting valve 32, or increase the circulation of gases to the combustion zone by more completely closing valve 13 and opening valve 14 more fully, or by introducing an additional amount of combustion supporting gas by opening valve 19, or by combinations of these adjustments, or by heating the raw fuel in 10 to a higher temperature by promoting combustion reactions therein using more oxygen introduced through 24. Another adjustment for accomplishing a similar result is to supply a combustion supporting gas by opening valve 8. To decrease the completeness of carbonization of the solids at about the bottom of zone 2 the opposite adjustments are made.

In case the temperature of the solids being 75 zone A, varying with the depth of zone A and

processed decreases too rapidly in zones C and 3 before they are sufficiently steamed, either introduce air (or more air) by opening valve 21, or raise the temperature of the fluidizing steam supplied through 22 and 23, or both. The rate of carbonization may be very rapid, hence the temperatures in zones A and B should be watched and the flow of solids in process regulated according thereto or the flow of fluids, particularly the combustion supporting fluids should be adjusted in accordance therewith.

For fluidizing solids varying from very fine-size in one case to very coarse in another case, the velocity of the fluidizing gas stream measured as in an empty carbonizer will vary respectively from about 0.1 to 10.0 feet per second. The velocity referred to at this point, and at other points in the specification, is superficial velocity; that is, the velocity which would obtain in the enlarged zone or reactor with a given inlet and outlet velocity if the enlarged zone or reactor were empty. When operating at low carbonizer capacity it is sometimes necessary to use an appreciable amount of recirculated gas and only a small amount of combustion supporting gas. In this case gas passing out of the carbonizer through 5 and 6 is recirculated back to the carbonizer preferably after removing condensable product; it is compressed to the necessary pressure and is supplied through valve 37. Actually very little heat is required, when the fuel is supplied dry, in addition to that carried away as sensible heat in the gas and solids, and it is possible to reduce these losses to small quantities. For example when zones C and 3 are deep, the solids may be discharged cool and steam at about 250° F. may be used. This effect is further facilitated by employing a deep zone C and incorporating another packed zone in it but spaced below zone 3.

Normally the pressure in the system is just sufficiently above atmospheric pressure to operate as described but with some carbonaceous solids the physical nature, porosity, density, etc. are appreciably affected by a change in pressure; hence this invention is not limited in this respect; it may be operated at high or low pressures. The density of the product made at high pressure is greater than that made at low pressures.

Referring again to the figure, the zones C and 3 are shown to have smaller diameter than A and B but this is not always necessary. The diameter is proportioned so that the velocity of the stream flow will fluidize the solids in zones C and 3. Because the volume of gaseous fluids flowing upwardly is greater in zones A and B than that in C and 3 it is advisable that the latter zones be of smaller diameter than the former zones, in order to obtain best results.

The actual time required to carbonize a fuel when the particles are say 60 to 200 mesh size is a variable depending on the moisture content of the fuel, volatile matter initially present therein and its temperature as charged as well as the velocity of flow and temperature of the gases passing upwardly through the bed. With a temperature of 1200° F. in zone A coal can be carbonized in zones A and 2 in a matter of seconds, 10 to 30 seconds being usually ample. However, operating variables may be adjusted to provide longer or shorter time when desired. A convenient rate of supply of dry coal to carbonizer 1 for carbonizing is 0.05 to 0.25 pounds per second per square foot of horizontal sectional area of

the temperature of the gas stream rising from zone 2 into zone A and the velocity of said stream. The overall duration of the carbonizing time (total time in the carbonizer) may be adjusted at will. Normally a convenient time is of the order of 20 to 60 seconds.

It will of course be understood that the carbonizer can be operated without the de-ashing unit when desired. In this event either chamber 10 can be considered as a reservoir or the feed for the fuel carbonizer can come directly from conduit 34 and through valve 33. In this case consider valve 14 closed and the gases for zone 17 are supplied through valves 19 and 37.

One skilled in the art will recognize that the procedures outlined herein and modifications of them will be applicable in making low-temperature coke, high-temperature coke, in the pyrolysis of oil shale, and in general in heat-treating finely divided solids particularly carbonaceous solids. Magnesium carbonate gives up  $\text{CO}_2$  at  $350^\circ \text{C}$ . and calcium carbonate decomposes at  $825^\circ \text{C}$ .; these products may be calcined, in a fine state of division in this manner. In this case air would be used as the bottom fluidizing agent and coolant and it would be preheated in traveling up through zones C and 3 and would be the combustion supporting fluid in zone 17, the fuel could be introduced through valve 37.

Having described our invention so that one skilled in the art can practice it, either as described or with modifications, we claim:

1. The continuous process of carbonizing carbonizable solids which comprises forming a deep single substantially continuously downwardly moving bed of finely divided carbonized solid fuel in an upright carbonizer, continuously feeding the carbonizable solid in finely divided state to the upper part of said bed, maintaining said bed in a fluidized condition by passing upwardly therethrough a stream of gas comprising, near the lower part of said bed, steam introduced at that point and, at a higher level in said bed, steam, combustion supporting gas and gaseous combustion residues, causing said bed in its downward travel to pass through the interstices of large size bodies maintained as a pack in two separate zones in the path of said bed, said packs preventing back-mixing of the finely divided solid upwardly through said zones into preceding portions of said bed, introducing the combustion supporting gas into said bed between said zones, recovering from above said bed vaporous products of

the carbonization of said carbonizable solid and recovering carbonized solid from the lower portion of said bed below the point of introduction of steam into said bed, the flow of materials and the feed of steam and combustion supporting gases being so regulated that throughout the upper portion of the bed above the upper packed zone, the finely divided material is maintained at a carbonization temperature above the plastic range of said carbonizable solid and between  $900$ – $1400^\circ \text{F}$ ., in the next lower zone including the upper packed zone, the finely divided material is maintained at a temperature between about  $1600$ – $2000^\circ \text{F}$ ., and in the lowermost zone, including the lower packed zone, said material is quenched with steam.

2. In the process defined in claim 1, the step of introducing a small amount of a combustion supporting gas along with the steam.

3. The process as defined in claim 1, in which the solids are fuel selected from the class consisting of lignite, sub-bituminous coal, bituminous coal, semi-bituminous coal, and anthracite coal.

4. A method according to claim 1 in which the finely divided carbonizable solid fed to the carbonizing zone is subjected to a preliminary treatment for the removal therefrom of ash constituents.

5. A method according to claim 1 in which the combustion in said next lower zone is at least in part the combustion of combustible gases produced by the reaction between steam and hot carbon in the quenching zone.

WILLIAM W. ODELL.  
GEORGE L. MATHESON.

#### REFERENCES CITED

The following references are of record in the file of this patent:

#### UNITED STATES PATENTS

| Number    | Name          | Date           |
|-----------|---------------|----------------|
| 1,639,356 | Wallace       | Aug. 16, 1927  |
| 1,923,918 | Davis         | Aug. 22, 1933  |
| 1,927,459 | Krczil        | Sept. 19, 1933 |
| 1,955,025 | Salbel et al. | Apr. 17, 1934  |
| 2,148,827 | McFarland     | Feb. 28, 1939  |
| 2,162,763 | Stuart        | June 20, 1939  |
| 2,444,990 | Hemminger     | July 13, 1948  |

#### OTHER REFERENCES

Bureau of Mines R. I., 3,711, May, 1943.